

## UNITED STATES PATENT OFFICE

1,943,347

## SPRING STEEL

Joseph Kent Smith, Detroit, Mich., assignor to  
 The Beryllium Corporation, New York, N. Y.,  
 a corporation of Delaware

No Drawing. Application August 10, 1931  
 Serial No. 556,324

## 2 Claims. (Cl. 75—1)

This invention relates to a series of compositions of steel characterized by high tensile strength, great flexibility and extremely high fatigue resistance, the essential feature of all members of the series being the presence of metallic beryllium, always in quantities less than 5% of the total, and preferably less than 1% of the total.

In addition to iron and carbon, present in all steels, and the beryllium which is the parent alloying substance of my invention, I have found it necessary, for best results, to add one or more of the metals chromium and molybdenum. While I do not mean to be limited to such compositions, I have found that when molybdenum is used, best results are obtained when the carbon content is kept under 0.80%. Similarly, when chromium alone is present without any molybdenum, the carbon had best not exceed 0.70%, and when both molybdenum and chromium are present in the alloy, carbon of 0.50% had best not be exceeded.

The usual steel constituents, manganese and silicon, are, of course, also present, the manganese frequently rising into the range of 1.0% to 1.5%, where it, too, may be considered an alloying element. The steels of the series of my invention lend themselves readily to substantially

the heat treatment standard for steel of the corresponding carbon content.

One simple example of the invention is a spring steel of the composition for which the invention is especially useful.

|            | Per cent |
|------------|----------|
| Carbon     | 0.35     |
| Chromium   | 1.00     |
| Molybdenum | 0.35     |
| Manganese  | 1.00     |
| Beryllium  | 0.30     |

In general, chromium, molybdenum and manganese are best held under 1.5% each.

## I claim:—

1. Spring steel comprising carbon approximately 0.35%, chromium approximately 1.00%, molybdenum approximately 0.35%, manganese approximately 1.00% and beryllium approximately 0.30%, and the balance iron.

2. A steel comprising from about 0.30% to about 5% beryllium; about 0.35% but not more than 1.5% molybdenum; about 1% but not more than 1.5% chromium; about 0.35% but not more than 0.50% carbon; about 1% but not more than 1.5% manganese; and the balance iron.

60

80

85

90

95

100

105

30

35

40

45

50

JOSEPH KENT SMITH.